

Oct. 21, 1924.

1,512,371

W. H. SOMMER

PROCESS OF COATING MATERIAL

Filed March 25, 1922



INVENTOR.  
*William H. Sommer*  
BY  
*Charles L. Post*  
ATTORNEYS.

## UNITED STATES PATENT OFFICE.

WILLIAM H. SOMMER, OF PEORIA, ILLINOIS.

## PROCESS OF COATING MATERIAL.

Application filed March 25, 1922. Serial No. 546,933.

*To all whom it may concern:*

Be it known that I, WILLIAM H. SOMMER, a citizen of the United States, a resident of Peoria, in the county of Peoria and State of Illinois, have invented new and useful Improvements in Processes of Coating Materials, of which the following is a specification.

This invention has reference to a method 10 of coating materials having an iron base and particularly the coating of wire used in the fence industry and for other purposes.

The principal object of this invention is to permit the formation of heavily coated 15 material and obviating the use of long coating baths. Such formations of heavy coatings has for its object an improved coating which will be more resistant to atmospheric rusting and corroding conditions than is ordinary galvanized wire, and which further 20 will permit a heavier coated wire to be used in wire fabricating machines without causing the coating to crack or flake off as is the case with heavily coated wire coated by ordinary processes.

A further object of the invention is to permit the use of higher speeds for galvanizing wire, and, at the same time, causing a heavier coating to be formed on the wire than 30 can be used under the ordinary galvanizing processes where heavier coatings are desired.

Galvanized wire which is to be used for fabricating purposes and more particularly that which is to be used in the manufacture 35 of woven wire fencing must have a relatively heavy coating of spelter in order to be able to withstand atmospheric corroding conditions, and before my invention was developed this was not possible except at a much increased cost of production, due to 40 slow speeds, long spelter baths and other causes.

At the present time there are only two methods in use whereby these necessary 45 heavy zinc (spelter) coatings may be obtained by the hot process of galvanizing. The first method is to pass the wire very slowly as it emerges from the galvanizing bath, thru finely divided charcoal. By such 50 a process a smooth, thick coating may be obtained. This method is used for the manufacture of telephone wire. It has serious drawbacks, however, from an economic standpoint, because the wire must travel at a very slow speed, a very high grade zinc 55 must be used, and, furthermore, the coated

wire cannot be subjected to the action of wire-fence fabricating machines without having considerable of the zinc coating crack or flake off the iron base. The second method is to cause the wire to travel at relatively slow speeds, through a bath of molten spelter, the speed depending on the gauge of the wire, the thickness of the coating desired and the length of the molten spelter bath, and wiping the wire by passing it between suitable wipers. This process, too, has its economic drawbacks, because of the slow speeds required, the long spelter baths necessary and the consequent attending losses from dross and oxide (skimming) formations.

I have discovered that if instead of wiping the wire as soon as it leaves the spelter bath, as is the case in ordinary hot galvanizing processes, I wipe the wire at a substantial distance from the point where the wire leaves the coating bath, I obtain a heavier coating on the wire and the coating is also smooth. It is necessary that this wiping take place before the coating has set, otherwise I do not obtain a perfectly smooth coating. For this reason the location of the wipers is dependent on the size of the wire, the speed at which it travels and the temperature of the spelter.

I have further discovered that by passing the wire thru an insulated medium I can keep the coating fluid for a longer length of time than is the case if I cause it to pass directly from the spelter to the wipers thru the air. Consequently, I preferably pass the wire as it leaves the spelter upward thru an insulated tube, then downwardly thru another insulated tube and then thru suitable wipers.

In the accompanying drawing there is illustrated diagrammatically so much of a continuous galvanizing or coating apparatus to illustrate the use of the invention, including "acid" bath, "flux" bath, a "drier", a "coating bath", and an insulated tube through which the coated wire is passed before the wiping action, and finally a "wipe" of any suitable or preferred construction.

For example, I have taken a No. 9 gauge wire and passed it thru about thirteen to fifteen feet of spelter held at a temperature of approximately 875 degrees F. and passed it between asbestos pressure wipers immediately. This coating would stand two tests in copper sulfate before failure. Another

- similar wire treated in exactly the same manner, but interposing approximately three feet between the wipes and the point where the wire emerged from the spelter gave a 25
- 5 coating which would stand from three to four copper sulfate tests. The same result would occur when the insulator was used, this being particularly effective for the smaller wires. The speed of the wire in 10 the above cases was approximately 80 feet per minute. If instead of traveling at the rate of 80 feet per minute the wire had been traveling at the rate of 100 feet per minute, the wipes instead of being three feet from 15 the point at which the same emerged from the spelter could have been approximately four feet distant. An essential factor in this process is the temperature of the coating bath which must be substantially higher 20 than the melting point of the coating material, as for example in the case of spelter the minimum temperature in order to obtain the best results should not be below 850 degrees F.
- 25 I realize, of course, that wiping wire is old, but the method by which I secure my heavy coatings is new and it is obvious that modifications of the disclosed process may be made without departing from the spirit 30 and scope of the invention.
- What I claim is:
1. The process of galvanizing wire, which consists in passing the wire, first—through a molten spelter bath and then passing the 25
  2. The process of coating materials having an iron base, which consists in subjecting the same, first—to a molten coating bath— 40 then passing the same thru a heat insulator, and finally wiping the coating while in a heated state. 45
  3. The process of galvanizing wire, which consists in subjecting the wire to a molten coating bath, then passing the coated wire through a heat insulator and wiping the coating just prior to the solidification of the coating. 50
  4. The process of galvanizing wire, which consists in subjecting the wire to a coating bath of approximately 875 degrees F., and wiping the coating at approximately three feet from the point where the wire is removed from the bath, such wire being moved 55 continuously and at approximately 80 feet per minute. 55
  5. The process of coating materials having an iron base, which consists in subjecting the material to a molten coating bath, then passing the coated material thru a heat insulator, and wiping the coating just prior to the solidification of the coating. 60

In witness whereof I have hereunto affixed my hand this 18th day of March, 1922.

WILLIAM H. SOMMER.